

Patented Sept. 26, 1922.

1,430,115

# UNITED STATES PATENT OFFICE.

RALPH E. RINDFUSZ, OF NORTHAMPTON, AND VANDERVEER VOORHEES, OF HOLYOKE, MASSACHUSETTS, ASSIGNORS TO AMERICAN WRITING PAPER COMPANY, OF HOLYOKE, MASSACHUSETTS, A CORPORATION OF NEW JERSEY.

## PROCESS FOR RECOVERING FLAX FIBER.

No Drawing.

Application filed November 15, 1919. Serial No. 338,299.

To all whom it may concern:

Be it known that we, RALPH E. RINDFUSZ and VANDERVEER VOORHEES, citizens of the United States, residing at Northampton, 5 in the county of Hampshire, and Holyoke, in the county of Hampden, respectively, in the State of Massachusetts, have invented certain new and useful Improvements in Processes for Recovering Flax Fiber, of 10 which the following is a specification.

This invention relates to a process for recovering clean fiber from flax straw or flax tow.

The straw of the fiber flax plant is at 15 present subjected to an elaborate retting process for the isolation and recovery of fiber for use in the textile industry; and in the combing and carding operations necessary in the production of the clean 20 fiber, a by-product is combed out, consisting of a tangled mass of fiber and woody shives which is known as flax tow. Likewise in the threshing of seed flax, a slightly 25 different plant than fiber flax, for the recovery of seed, the straw by-product has been subjected to mechanical and chemical processes in order to remove in large part the woody shives from the straw and again produce a flax tow.

30 Flax tow is at present used in the upholstery arts and for similar purposes and if sufficiently refined by the removal of the objectionable shives is also used in the manufacture of fiber board, counter board, 35 heavy wrapping paper and the like.

As a general rule only the flax tow from the textile industry is of sufficiently good 40 quality for the manufacture of fiber-board, and since most of this material has been imported heretofore, which importation was stopped during the war, various attempts 45 have been made to refine the flax tow from the seed flax plant into suitable condition for use in fiber-board, etc. An account of these experiments has been published in 50 bulletin No. 322 of the United States Dept. of Agriculture, dated January 7, 1916 and entitled "Utilization of American Flax Straw in the Paper and Fiber-Board Industry."

In none of the prior processes or experiments has it been possible to remove or reduce all the shives from the fiber of the flax tow without impairing the strength

and usefulness of the fiber itself either for 55 paper making or other purposes. The prior workers in the art were compelled to be satisfied with a moderate degree of success which enabled them to sufficiently refine the fiber for heavy grades of paper and fiber- 60 board although a clean fiber entirely free from unreduced shives would have been highly prized as stock for high grade writing papers, parchment and pure linen papers.

65 The present invention therefore is for a method for cleaning substantially all of the shives or unreduced woody material from the fiber of the straw and for producing a fiber suitable for the manufacture of the 70 finest grades of writing paper as well as for textiles. An important chemical principle upon which the present invention is based is that cold nitric acid, i. e. at ordinary room 75 temperature, either alone or in combination with certain other acids, will not deleteriously attack the fiber of flax straw or tow but will attack and reduce the woody portion or shives, which, as is well known, comprise cellulose fibers associated with 80 encrusting or adsorbed lignin. In the application of this principle although nitric acid alone is effective, it has been found that sulphuric or hydro-chloric acid added to nitric in a cold mixture will improve the 85 action slightly and also that various other acid compounds of nitrogen may be employed for the reduction of the shives such, for instance, as nitrous acid, or a nitrite salt together with a suitable reagent for the 90 release of the nitrous acid. After the shives of the flax tow or straw have been reduced by the action of the nitric or nitrous acid and the cellulose fibers thereby set free, the gelatinous substance derived from the 95 lignin or other non-cellulosic components is easily washed and separated from the fiber by any of the well known alkali cooking and washing processes.

100 As a preliminary treatment, before subjecting the tow or straw to the nitric acid or its equivalent, it is preferred to cook the tow in one of the usual alkali compounds such as milk of lime, which will reduce a large part but not all of the shives. After 105 the alkali treatment the fiber should be washed thoroughly in water to remove alkali and products derived from the woody

material and then subjected to the nitric acid treatment. At the end of the acid treatment the fiber should be again washed to remove the acid and finally given another alkali cooking treatment this time preferably with a comparatively dilute solution of caustic soda to complete the removal of non-cellulosic shive material. Thereafter the fiber is washed clean in water and is ready for the bleaching agents and other operations in the manufacture of paper or textiles.

A more particular description will now be given of the steps at present preferred for carrying out this process although it will be understood that considerable variation in the mechanical devices, degree of temperature, duration of time and proportions of materials may be made and still obtain a satisfactory working of the process.

The flax fiber in the form of tow or straw is first cooked with 20% of its weight of milk of lime  $\text{Ca}(\text{OH})_2$ , which may be effected in a closed cylinder into which steam is introduced for heating the same. The steam is maintained at a pressure of about 50 lbs. for about three hours and the cylinder should be rotated slowly for the purpose of agitation.

At the end of this period the fiber is removed, drained of its alkali liquor and washed in water in a suitable washing machine or beater and then pressed dry.

The pressed fiber is then placed in an acid tank containing about 40% of the fiber weight, of a cold acid mixture made up of equal proportions by weight, of sulphuric acid,  $\text{H}_2\text{SO}_4$ , and nitric acid  $\text{HNO}_3$ , and is agitated in this cold acid mixture for about five hours. By a cold acid mixture is meant that the acids are kept at ordinary room temperatures approximately 70° F. An acid mixture containing equal proportions by weight of nitric acid and hydrochloric acid  $\text{HCl}$  may also be employed in this step in place of a mixture of nitric and sulphuric acids.

Furthermore, this acid treatment may, if desired, be effected with nitrous acid  $\text{HNO}_2$ , in which case the pressed washed fiber is placed in the acid tank with a solution containing 10% of the fiber weight of sulphuric acid  $\text{H}_2\text{SO}_4$ , and during the agitation a concentrated solution of sodium nitrate  $\text{NaNO}_2$ , containing 10% of the fiber weight of  $\text{NaNO}_2$ , is admitted at intervals to the bottom of the acid tank containing the acid and fiber. The reaction liberates nitrous acid to act on the shives of the fiber. The fiber is preferably agitated in this solution for about six hours and in this nitrous acid

treatment it is not so essential to prevent the acid mixture becoming heated slightly above ordinary room temperatures.

After the acid treatment the fiber is removed, drained and again washed in water in a suitable washing machine to free the fiber from acid.

Thereupon the fiber is again cooked in an alkali preferably in a closed cylinder with about 40 to 50 lbs. of steam pressure a suitable alkali for this step being caustic soda  $\text{NaOH}$  in proportion of about 5% of the fiber weight. The fiber is thoroughly agitated during this cooking process which is continued for about two hours.

At the end of the final alkali cook, the fiber is removed and again thoroughly washed in water after which it is ready for being bleached in the usual manner. The fiber will now be entirely free of unreduced shives and it will be found practically unimpaired in strength so that it is suitable both for paper and textile manufacturing processes.

The pulp prepared in the manner described above is quite free from unreduced shives and is suitable for the manufacture of high-grade white or tinted papers, with satisfactory yields from the original tow or straw. The treatment described is effective for the breaking down of the woody or shive material, and the isolation therefrom of the shive fibers; which latter remain to a large extent in the paper and may be readily identified therein, along with the bast fiber of the flax, by their characteristic forms and behavior toward fiber stains.

What we claim is—

1. Process of preparing high-grade paper pulp from flax tow, comprising subjecting the tow to an alkaline cook under super-atmospheric pressure to soften the shive material; removing the alkali and treating at substantially normal temperature with an acid solution comprising an oxy-acid of nitrogen; and completing the removal of ligneous shive material by a further alkaline treatment.

2. Process of preparing high-grade paper pulp from flax tow, comprising subjecting the tow to an alkaline cook under super-atmospheric pressure to soften the shive material; removing the alkali and treating at substantially normal temperature with an acid comprising sulfuric acid and an oxy-acid of nitrogen; and completing the removal of ligneous shive material by a further alkaline treatment.

RALPH E. RINDFUSZ.  
VANDERVEER VOORHEES.